

Nov. 30, 1948.

M. F. BOOTH

2,454,961

METHOD AND APPARATUS FOR CASTING ALUMINUM

Filed June 7, 1943

5 Sheets-Sheet 1



Nov. 30, 1948.

M. F. BOOTH

2,454,961

METHOD AND APPARATUS FOR CASTING ALUMINUM

Filed June 7, 1943

5 Sheets-Sheet 2

FIG. 2



FIG. 3



FIG. 4



FIG. 5



INVENTOR  
MORRIS F. BOOTH  
BY  
Toulmin & Toulmin  
ATTORNEY

Nov. 30, 1948.

M. F. BOOTH

2,454,961

METHOD AND APPARATUS FOR CASTING ALUMINUM

Filed June 7, 1943

5 Sheets-Sheet 3



INVENTOR  
MORRIS F. BOOTH  
BY  
Gouldman & Gouldman  
ATTORNEYS

Nov. 30, 1948.

M. F. BOOTH

2,454,961

METHOD AND APPARATUS FOR CASTING ALUMINUM

Filed June 7, 1943

5 Sheets-Sheet 4

**FIG. 14**



**FIG. 16**



**FIG. 15**



**FIG. 17**



INVENTOR  
MORRIS F. BOOTH  
BY  
Tschirhart & Tschirhart  
ATTORNEYS

Nov. 30, 1948.

M. F. BOOTH

**2,454,961**

THERMOPHILIC BACTERIA

## METHOD AND APPARATUS FOR CASTING ALUMINUM

5 Sheets-Sheet 5



INVENTOR  
**MORRIS F. BOOTH**  
BY  
**Toulmin & Baldwin**  
ATTORNEYS

## UNITED STATES PATENT OFFICE

2,454,961

METHOD AND APPARATUS FOR CASTING  
ALUMINUM

Morris F. Booth, Alden, Mich.

Application June 7, 1943, Serial No. 489,929

11 Claims. (Cl. 22—70)

1

This invention relates to casting or molding of metals, and particularly to a process and apparatus for the same wherein high pressure is maintained on the metal in the mold or die during the entire cooling process upon the metal that is cast or molded.

In the art of casting or molding metal, in what is termed the die casting art, it has been the common practice to melt a body of metal that is to be cast into a mold within a melting pot and to force the liquid metal into a suitable mold or die through a gooseneck or spout of many forms under pneumatic or hydraulic pressure. In all of these previous processes and apparatus for molding or die casting metal, the metal that is cast in the mold completely fills the spout of the die casting machine, the sprues, the runners, as well as the mold cavity. The conventional practice has been to cool the molds as quickly as possible by circulating cooling fluid through the same so as to reduce the operating time of each cycle of operation of the machine. Therefore, all parts of the mold have been intensely cooled to rapidly chill the metal that is cast into the mold cavity and permit the molds to be quickly opened after the metal has been cast.

While the art of die casting has reached a relatively high stage of perfection, yet articles that are produced by present day commercial die casting or molding methods are substantially limited in size because porosity of the metal is one of the major considerations, and one of the major difficulties of articles that are produced by conventional molding or die casting methods.

It is well-known that the wall thickness of articles produced by conventional die casting or molding purposes must be substantially greater than if the porosity of the metal could be completely eliminated, and that if the density of the metal could be increased during the die casting or molding process, the wall thickness could be considerably reduced.

It is, therefore, an object of this invention to provide a process and an apparatus for casting or molding metal under pressure in such a manner that pressure is constantly maintained on the liquid metal in the mold during the entire cooling period so that when a metal shrinks during the cooling period the pressure on the metal that is still in a plastic or a liquid condition will force it into various parts of the mold to absorb this shrinkage and fill in the mold cavity solidly, whereby the density of the metal cast or molded is greatly increased and the porosity is substantially eliminated.

Another object of the invention is to provide

2

a process and an apparatus for casting or molding metals in their liquid state under pressure that is constantly maintained on the entire body of unsolidified metal within the mold cavity during the entire cooling period.

Still another object of the invention is to provide a process of molding or casting metals in the liquid state under pressure that is constantly maintained on the unsolidified body of metal in the mold or die wherein the body of metal in the die is cooled in such a manner that the body solidifies gradually from the remote portions of the mold cavity toward the opening through which the mold has been filled so that the metal adjacent the mold opening will be the last portion of the body of metal within the mold cavity to solidify, whereby the pressure that is maintained on the metal in the filling opening will be constantly transmitted throughout the body of metal in the die or mold as it is cooling and thereby increase the density of the metal as it is cooling in the mold and substantially eliminate porosity in the cast body of metal.

Another object of the invention is to provide a process of casting or molding metal in a liquid state in such a manner that the metal to be cast is moved into the mold by means of a carrier metal that has a lower melting temperature than the metal that is being cast so that the carrier metal will at least partially enter the mold or die and thereby constantly maintain pressure upon the metal that is being cast during the cooling period irrespective of the shrinkage of the cast metal during the cooling period because the molten carrier metal can follow any shrinkage contour developed by the surface of the metal being cast.

Still another object of the invention is to provide a process of casting metal under pressure in accordance with the foregoing object wherein the cooling of the cast metal is controlled in such a manner that the body of cast metal cools gradually from the portions thereof remote from the filling opening of the mold toward the filling opening whereby the carrier metal may constantly maintain pressure on the entire body of unsolidified metal during the entire cooling period and cause the unsolidified metal to be continually forced outwardly against the body of solidified metal until the body of metal being cast has completely solidified.

Another object of the invention is to provide a process for casting metals in a liquid state under pressure in accordance with any of the foregoing objects wherein a predetermined and selected quantity of metal is cast into a mold cavity.

55

Another object of the invention is to provide a process of casting or molding metal in a liquid state that is maintained under continuous hydraulic pressure during the entire cooling period wherein a mold or die is substantially filled with the metal to be cast or molded and a molten metal having a lower melting temperature than the metal that is being cast fills the remaining portion of the mold or die and has pressure applied thereon so as to produce hydraulic pressure upon the metal being cast and wherein the cooling of the cast metal is controlled in such a manner that the body of cast metal cools from those portions of the mold that are remote from the filling opening toward the filling opening so that the hydraulic pressure produced upon the cast metal will be maintained upon the entire body of unsolidified metal during the cooling operation and until the cast metal has completely solidified, whereafter the molten metal producing the hydraulic pressure can be removed from the portion of the mold that it fills, or at least substantially so.

Another object of the invention is to provide a process for casting or molding metals in a liquid state under pressure in accordance with any of the foregoing objects wherein hydraulic pressure is applied upon the metal being cast by means of a second metal having a lower melting temperature than the metal being cast.

Another object of the invention is to provide a process for casting metal in accordance with any of the foregoing objects wherein the metal being cast is of a different density than the low temperature metal that applies hydraulic pressure upon the cast metal.

Still another object of the invention is to provide a process of casting metal in a liquid state in accordance with any of the foregoing objects wherein the metal being cast may be supported upon the lower temperature metal which thereby acts as a carrier metal to move the metal to be cast into a mold.

It is another object of the invention to provide a process of casting metals in a liquid state under constant pressure wherein the carrier metal is a heavier metal than the metal to be cast.

It is another object of the invention to provide a process of casting metals in a liquid state under constant pressure wherein the carrier metal is lighter than the metal to be cast.

Another object of the invention is to provide an apparatus for practicing the process of this invention wherein the mold is retained in closed position by means of fluid motors and a fluid motor is provided for applying pressure upon the low temperature metal whereby it can apply hydraulic pressure upon the metal being cast.

Another object of the invention is to provide a process for die casting wherein more or less conventional molds can be used but wherein the principles of this invention can be practiced.

Still another object of the invention is to utilize the principles of this invention in practicing an extrusion process for forming metal articles of substantial length.

Still another object of the invention is to provide an extrusion process wherein molten metal is extruded by means of the application of hydraulic pressure upon the body of molten metal to force the same through an extrusion die.

It is still another object of the invention to provide an extrusion process wherein molten

metal has hydraulic pressure applied thereon for moving the molten metal through a cooling chamber and through an extrusion die so that the metal is gradually cooled from a liquid to a solid condition over a substantially long passage whereby the metal receiving chamber for molten metal may be intermittently refilled and the hydraulic pressure applied upon the molten metal intermittently without detrimentally effecting the metal being extruded because of the resiliency of the metal in a portion of the cooling chamber wherein the metal is in what may be termed a slush or spongy state.

Further objects and advantages will become apparent from the drawings and the following description.

In the drawings:

Figure 1 is a vertical cross sectional view of an apparatus upon which the principles of this invention can be practiced, and showing a diagrammatic hydraulic system for actuating the same.

Figure 2 is a diagrammatic illustration of the machine shown in Figure 1 illustrating the first step in the process in casting or molding using the principles of this invention.

Figure 3 is a diagrammatic view similar to Figure 2 showing the mold in closed position and with the cast metal in the mold and before any cooling of the cast metal has occurred.

Figure 4 is a diagrammatic view similar to Figure 3 illustrating the principles of this invention at work wherein the cast metal has started to cool and solidify within those portions of the mold cavity that are remote from the filling opening of the cavity.

Figure 5 is a diagrammatic view similar to Figure 4 illustrating the manner in which the final cooling of the cast metal takes place so that hydraulic pressure of the low temperature metal can be constantly maintained on the cast metal until it has completely solidified.

Figure 6 is a diagrammatic illustration of the use of the process of this invention, showing a part of the machine in cross section, wherein a metal disc has been placed upon the carrier metal to prevent agitation between the carrier metal and the casting metal when the casting metal is poured upon the carrier metal.

Figure 7 is a cross sectional view taken along line 7—7 of Figure 6.

Figure 8 is a diagrammatic view similar to Figure 6 showing the final stages of cooling of the casting metal wherein the carrier metal retains hydraulic pressure on the casting metal.

Figure 9 is a diagrammatic view similar to Figure 6 showing the manner in which a more dense metal can be carried by a light metal for casting or molding purposes.

Figure 10 is a view similar to Figure 8 showing the manner by which the light carrier metal maintains hydraulic pressure on the heavy casting metal during the final stages of cooling of the casting metal.

Figure 11 is a diagrammatic view similar to Figure 6 showing the manner by which chemical reaction, or alloying between the metals can be substantially prevented.

Figure 12 is a diagrammatic view similar to Figure 10 illustrating the final cooling period of the light metal that is forced into the mold by a heavier metal and the manner by which hydraulic pressure can be maintained upon the light metal during the final cooling period.

Figure 13 is a diagrammatic illustration par-

tially illustrating a complete machine similar to that shown in Figure 1 wherein hydraulic pressure can be maintained upon a casting metal in a slightly modified processing arrangement than disclosed in Figure 1.

Figure 14 is a vertical cross sectional view somewhat diagrammatically illustrating a machine by which the principles of this invention can be practiced in connection with die casting apparatus.

Figure 15 is a cross sectional view similar to Figure 13 illustrating the manner in which the mold is filled.

Figure 16 is an enlarged cross sectional view of a portion of the mold and nozzle engaged therewith shown in Figure 14 illustrating the location of the liquid level between the casting metal and the carrier metal.

Figure 17 is a cross sectional view of a mold wherein a plurality of articles are cast simultaneously illustrating the manner in which hydraulic pressure can be maintained upon each of the plurality of articles in a mold during the entire cooling period thereof.

Figure 18 is a cross sectional view of an apparatus, illustrating somewhat in diagrammatic form, for utilizing the principles of this invention as practiced in an extrusion molding process for extrusion molding metal articles for molten metal.

The machine upon which the process of this invention can be practiced consists of a frame 10 having the cored passages 11, 12 and 13 that are machined to receive the cylinders 14, 15 and 16, respectively. The cylinders 14, 15 and 16 receive rams 17, 18 and 19, respectively, that have the piston heads 20, 21 and 22, respectively, thereon that slidably engage cylinders 14, 15 and 16, respectively, whereby to form fluid motors. The end walls of the cylinders 14, 15 and 16 are closed by means of suitable closure wall members 23, 24 and 25, respectively.

The rams 17 and 18 carry mold or die members 26 and 27, each of which has a recess therein whereby to form a mold cavity 28 when the mold members 26 and 27 are in closed position as shown in Figure 1. The rams 17 and 18 thereby provide means for bringing the molds 26 and 27 into closed relationship, the molds being divided along the parting line 29, thus, the hydraulic motors 30 and 31 are arranged in opposed relationship.

A bed plate 32 is adapted to support the mold or dies 26 which slide upon the upper face 33 thereof when the molds are opened and closed. Also, the bed plate 32 supports the molds 26 and 27 when pressure is applied upon the top surface thereof by means of the ram 19 that extends from the hydraulic motor 34 to seal the lower faces of the mold members 26 and 27 upon the upper face 33 of the bed plate 32, whereby the mold members 26 and 27 are solidly held in engagement with the cylinder 35 that extends through the bed plate 32. An electric heating coil 36 is disposed around the cylinder 35 for maintaining the same at a relatively high temperature whereby to maintain molten metal therein in a molten condition as long as the metal is retained in the cylinder 35, in a manner and for reasons which will be herein-after described.

The mold members 26 and 27 are provided with cooling passages 37 and 38, respectively, for cooling the body of cast metal contained in the mold cavity 28, these cooling passages 37 and 28 being specifically arranged in the mold members 26 and 27 to cool the body of molten metal within the mold cavity 28 from the outside surface thereof

toward the filling opening, in a manner and for reasons which will be hereinafter described.

5 A second cylinder 39 extends from the cylinder 35 in axial alignment therewith. A cylinder bore 40 extends through the cylinders 39 and 35 in axial alignment with the mold filling opening 41 that is provided for the mold cavity 28 and is of substantially the same diameter as the cylinder bore 40, and for reasons which will be herein-after discussed.

10 The cylinder bore 40 receives a piston or a plunger 42 that is provided on the end of a ram 43 extending from the cylinder 44 of a hydraulic motor 45. The ram 43 being provided with a piston head 46 that reciprocates in the cylinder bore 41. A sealing closure wall member 48 is provided for the end of the cylinder 44.

15 The cylinder 44 is connected to the frame 10 of the machine by means of the strain rods 49, four of the strain rods being preferably provided around the cylinder 44. The cylinder 39 contains an electric heating coil 50 that is adapted to maintain the temperature of a metal contained within the cylinder 39 in a molten condition at all times.

20 The machine 10 may rest upon a suitable foundation 51.

25 The fluid motors 30, 31, 34 and 45 are preferably of the hydraulic type and a suitable source of fluid under pressure is provided for supplying these motors with operating fluid for reciprocating them in conventional manner. Any suitable type of pumping system may be provided for supplying the fluid under pressure, and since such pump systems for supplying fluid under pressure are well-known in the art, and the pumping system forms no part of this invention, no particular type of pumping system will be disclosed or described herein as any of the conventional forms of pumping systems can be used upon the machine of this invention.

30 In order to control the operation of the hydraulic motors 30 and 31, a 4-way valve 52 of conventional design is provided having a pressure supply conduit 53 that is connected to the pressure side of the pump for delivery of fluid under pressure to the valve 52. Conduits 54 and 55 are connected to opposite ends of the hydraulic motor 30 for supplying fluid under pressure thereto according to the setting of the 4-way valve 52 by means of the control handle 56. A return line 57 is provided on the 4-way valve 52 for returning fluid to a reservoir from one end of the motor 30 when fluid under pressure is being supplied to the opposite end of the motor 30.

35 The hydraulic motor 31 has a conduit 58 connected thereto that supplies pressure fluid to the advancing side of the hydraulic motor 31, this conduit 58 being connected to the conduit 54 that supplied pressure fluid to the advancing side of the hydraulic motor 30. A second conduit 59 connects the opposite end of the hydraulic motor 31, or the retraction side thereof, with the supply conduit 55 that conducts fluid to the retraction side of the motor 30. Thus, it may be seen that both hydraulic motors 30 and 31 are arranged in parallel circuit relationship for opening and closing the mold members 26 and 37, respectively.

40 A 4-way valve 60 is connected to a source of fluid under pressure by means of the conduit 61 whereby pump pressure is delivered to the 4-way valve 60 for delivery to either of the supply conduits 62 and 63 under control of the regulating handle 70. The conduit 63 is connected to the

advancing side of the hydraulic motor 44 while the conduit 62 is connected to the retraction or the push-back side of the hydraulic motor 44. A return line 65 is connected to the 4-way valve 66 for returning fluid from one side of the motor 34 to a reservoir when pressure fluid is being supplied to the opposite side of the motor.

A 4-way valve 66 is provided for controlling the operation of the hydraulic motor 45 and is connected to a source of fluid pressure by means of a conduit 67 whereby pressure fluid is delivered to the 4-way valve 66 for delivery into the supply conduits 68 and 69 under control of the handle 10. The conduit 68 is connected to the advancing side of the hydraulic motor 45 while the conduit 69 is connected to the retraction or push-back side of the motor. A return line 71 connects the 4-way valve 66 with a reservoir for delivering fluid thereto from one side of the hydraulic motor 45 when pressure fluid is being supplied to the opposite side of the hydraulic motor.

The process of pressure casting, and the apparatus for practicing the process, is particularly adaptable for casting large metal objects that have an individual unit weight of 50 lbs. to 75 lbs. or more. While the process of pressure casting of this invention may be used to advantage in pressure casting any size metal article, yet its special advantages are particularly meritorious when quantities of molten metal in units of 50 lbs. to 100 lbs. or more are handled for individual castings, such as cylinder heads of internal combustion engines. One of the particular disadvantages of pressure casting large metal products is the shrinkage of the metal that occurs during the cooling of the metal after it has been forced into a mold under pressure. In the usual form of pressure casting devices, and processes heretofore practiced, the procedure has been to attempt to follow the usual practice in connection with die casting of small objects wherein a metal was maintained in molten condition and forced through a gooseneck into the mold or die, the excess metal being drained off from the dies through the gooseneck after the metal object had cooled in the dies. While this general procedure is satisfactory for small articles wherein the shrinkage of the metal due to cooling is not great enough to cause any defect in the article, yet when large masses of a molten metal are pressure cast by the conventional methods it has not been possible to continuously maintain pressure on the casting metal in the mold during the entire cooling operation because the gates, sprues and runners contain the same metal that is being pressure cast so that these small cross sections of metal will freeze, or solidify, before the main body of the metal and thereby prevent any pressure which may be maintained on the sprue from being transferred into the main body of the metal cooling in the mold. Thus, when a large mass of metal is cast into a mold there has been no way of compensating for the shrinkage of the metal during the cooling period. This cooling of the metal when dealing with large masses of the metal is extremely vital because the large body will shrink sufficiently that a defective casting results due to a pulling away of a mold surface of a portion of the cast metal.

Therefore, according to the teachings of this invention, hydraulic pressure will be constantly maintained on a body of metal cast under pressure into a mold during the entire cooling period so that as the metal shrinks in the cooling and solidifying process the metal near the center of

the mold will be moved outwardly against the external portions that have cooled or solidified whereby the hydraulic pressure that is applied upon the metal within the mold will be continuous throughout the cooling operation.

The practice of the process of this invention is particularly disclosed in Figures 2 to 5, inclusive. In the practicing of this process a body of molten metal 72 is placed in the cylinder bore 40 and is maintained in a molten condition by means of the heating units surrounding the cylinder bore. This molten metal 72 is one that has a lower melting temperature than the metal to be cast, and preferably has a higher specific gravity than the metal to be cast so that this body of metal 72 may act as a carrier metal for moving a casting metal into the molds. The body of metal 72, of course, rests upon the plunger 42 extending from the hydraulic motor 45 so that when the plunger 42 is moved upwardly the molten body of metal 72 is carried upwardly thereby. In the specific example of this invention the body of molten metal 72 may be lead having a melting temperature of about 621° F. and has a specific gravity of 11.34.

The metal to be cast, as by way of specific example, may be aluminum having a melting temperature of about 1217° F. and a specific gravity of 2.7. In any instance, however, the metal that is to be cast will have a higher melting temperature than the carrier metal so that complete solidification of the casting metal can occur within the mold without any solidification of the carrier metal.

The casting metal, having the higher melting temperature, is poured into the cylinder bore 40 upon the surface of the carrier metal 72 in a molten condition. It is, of course, understood that the carrier metal 72 may be and preferably is above its melting temperature and is maintained at substantially the casting temperature of the casting metal, which in the case of aluminum shall be about 1217° F., to prevent heat absorption from the casting metal by the carrier metal.

The quantity of casting metal to be used will be relatively accurately gauged so that the casting metal will not quite fill the molds, that is the casting metal will not completely fill the filling opening 41 of the mold cavity 28. Sufficient casting metal is used to completely cast the desired article but in addition to this there is only a slight excess so that there will be a space left in the mold filling opening when the casting metal has been completely transferred from the cylinder bore 40 into the mold cavity 28. This arrangement is to permit the low temperature carrier metal 72 to rise into the mold filling opening 41 when the mold cavity 28 has been completely filled by the casting metal.

Therefore, as the first step in the process of pressure casting metals, a predetermined quantity of casting metal is placed within the cylinder bore 40 upon the carrier metal 72. This may be done by ladling a predetermined volume of molten casting metal upon the carrier metal as illustrated in Figure 2. It is, of course, understood at this time the molds 26 and 27 are in opened position to permit the casting metal to be poured into the cylinder bore 40. At this point it must be stated that lead and aluminum, the specific examples used in this instance do not mix, and that the specific gravity of aluminum is such that it will completely float upon the body of lead so that the aluminum that is

poured into the cylinder bore 40 will ride upon top of the surface of the lead carrier metal.

After the predetermined quantity of casting metal has been placed in the cylinder bore upon the carrier metal, the molds will be closed by means of the hydraulic motors 30 and 31, and the hydraulic motor 34 will retain the mold members 26 and 27 upon the bed plate 32 to seal the same against the cylinder 35. The hydraulic motor 45 is then advanced to move the plunger 42 upwardly thereby transferring the casting metal resting upon top of the carrier metal from the cylinder bore 40 into the mold cavity 28, as illustrated in Figure 3.

It will also be noted that, as previously mentioned, the casting metal, shown in light dotted lines, does not quite fill the mold filling opening 41 so that the carrier metal, illustrated in heavy dotted lines, will enter the mold filling opening. It is quite apparent that with both casting metal and carrier metal in a molten condition that the pressure applied upon the carrier metal by the plunger 42 will produce hydraulic pressure upon the casting metal 73.

Cooling fluid can now be circulated through the cooling passages 37 and 38 provided in the mold members 26 and 27 to begin cooling and solidifying the casting metal in a mold cavity 28. As previously mentioned the cooling passages 37 and 38 are arranged in the mold members 26 and 27 so that the cooling is first effective upon the cast metal in those portions of the mold that are most remote from the filling opening 41 thereof. This has been graphically illustrated in Figure 4 by indicating the solidified metal by the cross hatch lines in the upper portion of the mold cavity 28, which solidified portion of the metal is indicated by the numeral 73a. That portion of the metal indicated in small dots is that which is about ready to solidify and is stated to be in a slush or spongy condition. With the heat being constantly applied upon the cylinder 35 by means of the heating coils 36 and 50 the carrier metal, or lead, may be maintained in a molten condition.

From the illustration, shown in Figure 4, it will be apparent that as long as pressure is applied in an upward direction, as indicated by the arrow on the plunger 42 that the carrier metal 72 will constantly apply hydraulic pressure upon the casting metal 73 that is still in a molten condition within the interior of the mold cavity, thereby producing a dense casting structure while the casting metal adjacent the periphery of the mold begins to cool and solidify. It is, of course, understandable that the more pressure applied upon the plunger 42 the more dense will be the casting metal within the mold cavity 28.

As the cooling and solidifying of the casting metal proceeds, solidification will be gradually from the outside portions of the mold cavity 28 toward the filling opening 41 whereby that portion of the casting metal that is within the filling opening 41 will be the last metal to solidify. As illustrated in Figure 5, the casting metal 73a has solidified throughout the mold cavity with the exception of that small portion immediately adjacent the mold filling opening 41. It will, therefore, become apparent that with the metal solidifying from the outside extremities of the mold cavity toward the filling opening that the hydraulic pressure applied upon the casting metal by the carrier metal will be continued throughout the entire cooling period.

The product that is being formed as illus-

trated in this invention may be a cylinder head for an internal combustion engine and therefore the casting may contain as much as 50 lbs. to 75 lbs. of casting metal. Such a mass of casting metal has considerable shrinkage. This shrinkage has been the major problem in connection with the pressure casting of molten metals.

In the application of the process of this invention, however, it will be apparent that since the casting metal cools from the outside periphery of the mold toward the filling opening, thereby always retaining liquid metal toward the center of the casting that will be engaged by the carrier metal, that hydraulic pressure can be continuously applied upon the casting metal as it is solidifying, whereby the natural and normal shrinkage that occurs during the solidifying of the metal can be compensated for, and the metal in the center of the casting is therefore forced outwardly against the solidified metal continuously until the last portion of the casting metal has solidified. When the last part of the casting metal has solidified there will be a recess in that portion of the casting that is in the filling opening. However, this part of the article will have been designed so that the machining operation will remove this irregularity from the article, and also any alloying that has occurred between the lead and the aluminum will be retained in this portion of the casting that will be machined from the cast article so that the pure aluminum will have been cast within the article itself.

The plunger 42 is adapted to reciprocate within that portion of the cylinder that is always engaged by the carrier metal, which in this instance is the lead. It is well-known that the high temperature metals such as aluminum, brass, bronzes and others attack the walls of the chamber into which they are poured so that after a certain period of time the walls become pitted.

Therefore, in order to prevent the plunger from being damaged by the pitted walls, or to prevent leakage from around the plunger, the quantity of carrier metal in the cylinder will be such that the stroke of the plunger 42 will always be in the area that has been engaged by the low temperature carrier metal. If for any reason it becomes desirable, the walls of a portion of the cylinder may be recessed to a larger diameter than the plunger so that the plunger could operate within area that would be engaged by the high temperature casting metal. In this latter instance any pitting of the cylinder walls would not effect the plunger because there would be a space between the plunger and the cylinder wall. However, it will be understood that the lower portion of the cylinder will be engaged in a sliding relationship by the plunger and therefore acts as a guide means for the same and to seal the lower end of the cylinder.

It is a well recognized fact that liquids of different specific gravities can be made to float upon one another if they are carefully poured upon one another so that even though the liquids will intermix when agitated, that they will stay in layers as long as unagitated. However, as long as there is no agitation liquids of different specific gravities will form definite layers upon one another. This natural phenomenon has been taken advantage of in the practice of this invention which has already been made apparent by this specific illustration by the floatation of aluminum having a specific gravity of 2.7 upon lead that has a specific gravity of 11.34. It is quite apparent that other metals may be floated upon the lead as long as the specific gravity is less than the

specific gravity of lead, such examples being magnesium of a specific gravity 1.74, the brasses and bronzes having specific gravities from 7.5 to 8.95, the cast and gray irons having specific gravities from 7.03 to 7.13, and many others. It is, of course, understood that in all instances the carrier metal must have a vaporization point substantially above the melting temperature of the casting metal. In all of the previous examples the melting temperatures of metals are below the vaporization point of lead which is about 2960° F. Also, the melting temperature of the lead is substantially below the melting temperatures of the other metals, the melting temperature of magnesium being about 1203° F., of the brasses and bronzes from 1625° F. to 2235° F. and the cast and gray irons from 1960° F. to 2200° F. It is, of course, understood that many of the metals, or alloys of the metals can be used as the carrier metal as long as the specific gravity of the carrier metal is different from the specific gravity of the casting metal and the melting temperature of the carrier metal is below the melting temperature of the casting metal. This latter feature being important in order to permit the carrier metal to be drained from the mold filling opening after the casting metal has solidified in the mold.

In order to reduce the effect of alloying between the carrier metal and the casting metal, and to prevent agitation at the surface of the carrier metal when the casting metal is poured upon the same and thereby prevent agitation which would tend to produce intermixing and alloying of two metals, there is shown in Figures 6 and 7 a metal disc 75 that is positioned in the cylinder 35 and is floated upon the carrier metal 72. The top view of the disc is shown in Figure 7 which illustrates that the disc 75 is a loose fit within the cylinder 35, having the clearance 76 therebetween, whereby the disc 75 freely floats upon the carrier metal. The disc 75 is provided with one or more recess portions 77 that will permit the carrier metal to move above the disc 75 as illustrated in Figure 8.

When the casting metal is poured into the cylinder bore 40 it will thus strike the disc 75 and prevent any agitation between the two metals at the surface of the carrier metal. The casting metal may then be transferred into the mold in a manner as heretofore described, and in this latter instance the disc 75 will stop at or below the mold filling opening 41, as illustrated in Figure 8. The carrier metal 72 may then pass through the recess portions 77 in the disc 75 to complete the filling of the filling opening 41 in a manner heretofore described and maintain hydraulic pressure upon the casting metal during the entire cooling period for the same. When the plunger 42 is retracted the carrier metal will, of course, drop into the cylinder bore 40 and the disc 75 will again float upon the surface of the carrier metal.

In Figures 9 and 10 there is illustrated a reversal of the process heretofore described, wherein the carrier metal 78 has a lower specific gravity than the casting metal 79. In this instance, a metal disc 80 is placed within the cylinder bore 40 and is a sliding fit therewith, and in fact the disc may be slightly flanged in order to improve the engagement between the wall of the disc and the cylinder wall 40.

The disc 80 will be placed within the cylinder bore 40 upon the surface of the carrier metal 78

before the casting metal 79 is pored into the cylinder bore 40.

When the plunger 42 now moves upwardly to transfer the more dense casting metal 79 into the mold cavity 28 formed by the mold members 26 and 27, the casting metal 79 will be carried upwardly by means of the disc 80. In this instance, however, the disc 80 is constructed from a relatively thin sheet of metal.

10 The cooling of the casting metal 79 within the mold cavity 28 will proceed as heretofore described so that as the metal begins to shrink due to solidification there will be need for a movement of the unsolidified casting metal outwardly against the casting metal that has solidified to maintain the pressure upon the entire body of metal in accordance with the practice of the process heretofore described. Since pressure is being applied upon the carrier metal 78 by 20 means of the plunger 42, the disc 80 being a thin material, will bend upwardly when the metal above it solidifies, or moves outwardly toward the outer periphery of the mold so that the hydraulic pressure applied upon the metal disc 80 will thus be transferred to the casting metal 79 as illustrated in Figure 10. This bending of the disc 80 will continue throughout the entire cooling period as long as the casting metal shrinks and it is necessary for the carrier metal 78 to move upwardly 30 into the mold filling opening for constantly maintaining hydraulic pressure upon the casting metal. It will, of course, be understood that the cooling of the casting metal in this last instance is affected in the same way as heretofore described. When the molds are opened the carrier metal 78 will drop from the mold filling opening leaving the metal disc in the casting which can be machined off of the casting.

As an example of the metals that can be used 40 in this latter instance, aluminum having a specific gravity of 2.7 with a melting temperature of 1217° F. can be used as the carrier metal while some of the brasses and bronzes having specific gravities of 7.5 to 8.95 with melting temperatures of 1625° F. to 2235° F. can be used as the casting metal. It is, of course, understood that in this latter instance that the cylinder within which the plunger operates will be constructed from a material that will not be readily attacked by the high temperature metals, such cylinder being constructed from a silica iron or the like, or may have a quartz liner in the same.

Many of the metals have a great affinity for 45 one another and alloying proceeds very easily when they are in a molten condition. This is particularly true with the affinity of the brasses and bronzes for tin and zinc so that under these circumstances it may be desirable to prevent any direct contact of the metals with one another at the time the casting metal is poured into the cylinder. This condition is true whether the casting metal is a light or a heavy metal and whether the carrier for the casting metal is more dense or less dense than the casting metal. The 50 arrangement just previously described would be satisfactory to prevent such alloying between the metals, but is illustrated in Figures 11 and 12. A flat thin disc 81 positioned within the cylinder bore 40 may be sufficient to prevent the alloying 55 of the metals. The disc 81 will bend to conform to the shape of the casting as it shrinks which is illustrated in Figure 12, and as particularly described with regard to the disc 80 illustrated in Figure 10.

70 In Figure 13 there is illustrated a slightly modified

fled arrangement for practicing the process of casting metal under pressure and for constantly maintaining hydraulic pressure on the casting metal as it is cooling within a mold. The general arrangement of the machine may be substantially as heretofore described with regard to Figure 1 wherein the mold members 82 and 83 are supported upon a bed plate 84 and are moved toward one another by means of the rams 17 and 18 that extend from the hydraulic motors 30 and 31. The mold members 82 and 83 engage one another along the parting line 85. The ram 18 carries a platen 86 that engages the molds 82 and 83 to close the mold cavity 87 and to retain the molds against the bed plate 84 so as to seal the mold 82 against the upper end of the cylinder 88 that has a cylinder bore 89 for receiving a body of material 90 that has a melting temperature that is below the melting temperature of the casting metal that is placed within the mold cavity 87.

In this arrangement the mold cavity 87 has the filling opening 91 extending through the top walls of the mold members 82 and 83 so that the mold cavity 87 can be filled directly by ladling a predetermined quantity of casting metal into the mold cavity. The mold members 82 and 83 are provided with cooling passages 92 and 93, respectively, that are positioned about the mold cavity 87 in such manner that the casting metal within the mold cavity 87 cools from the outer extremity of the mold cavity 87 toward the filling opening 91 in the same manner as heretofore described with regard to the operation of the machine, as illustrated in Figure 1.

A fluid passage 94 extends upwardly through the mold member 82 and connects with the cylinder bore 89. The passage 94 has a horizontal portion 95 that is provided with a downwardly slanting wall 96 so that any liquid in the passages 94 and 95 will return to the cylinder bore 89 when the plunger 42 is in its downward position.

Cooling passage 97 may be provided in the platen 86 above the filling opening 91 for reasons which will hereinafter become apparent.

When producing a casting in the apparatus just described with regard to Figure 13, the molds 82 and 83 will first be closed by operating the hydraulic motors 30 and 31. A predetermined quantity of casting metal will then be introduced into the mold cavity 87 to fill the same to the approximate level indicated by the liquid level 98. The platen 86 will then be brought down upon the mold members 82 and 83 thereby closing the mold filling opening 91, the hydraulic motor 34 being operated for this purpose.

The metal within the cylinder bore 89 will have a lower melting temperature than the casting metal that has been introduced into the mold cavity 87, this metal being retained in a molten condition at all times by means of the electric heating coil 99 that is provided in the wall of the cylinder 88. Also, the body of metal 90 will be a lighter metal than the casting metal that has been poured into the mold cavity 87. As a specific example, the pressure metal 90 may be zinc having a melting temperature of about 786° F. and a specific gravity of 7.4 while the casting metal may be one of the brasses or bronzes having a melting temperature of 1625° F. to 2235° F. and with specific gravities of 7.5 to 8.95. It will, therefore, be seen that when the zinc is transferred through the passages 94 and 95 into the space 100 above the casting metal in the mold cavity 87 that it will float thereon due to the

difference in these specific gravities of the metals.

Since the molds 82 and 83 are now closed and the platen 86 has been brought into engagement therewith, the hydraulic motor 46 may advance the plunger 42 to transfer the molten pressure metal 90 through the passages 94 and 95 into the space 100 in the mold cavity 87 whereby hydraulic pressure will be applied upon the surface 98 of the casting metal. As previously described, the cooling of the casting metal in the mold cavity 87 will proceed from the outer extremities of the mold toward the filling opening, so that the filling opening will be the last portion of the casting metal to solidify. Since the pressure metal 90 has a lower melting temperature than the casting metal it will remain fluid throughout the entire cooling period and maintain hydraulic pressure upon the surface of the casting metal irrespective of the contour that is finally developed in the surface of the casting as a result of the shrinkage of the casting metal during the cooling process.

After sufficient time has elapsed to permit complete solidification of the casting metal in the mold 87, the plunger 42 will be retracted whereby to permit the pressure metal in the passages 94 and 95, and in the upper portion of the space 100 to return into the cylinder bore 89 so that it can be used again on the next cycle of operation.

It will be noted that at this time there will be a small amount of pressure metal that will have remained in the space 100 that will be entrapped in the cavity 101 produced in the surface of the casting as a result of the shrinking of the casting metal during the cooling process. Therefore, at this time cooling fluid can be circulated through the passages 97 provided in the platen 86 so as to solidify the pressure metal that has been entrapped in the recess 101 before the casting is removed from the mold whereby to prevent spilling of any hot metal when the molds are opened.

As previously described the portion of the casting that contains the recess is machined from the casting so that any pressure metal that might remain in this recess will not appear in the finished article.

It will, of course, be necessary to make up periodically for the loss of the pressure metal in the cylinder 88, but small pieces of metal can be periodically introduced into the cylinder 88 to make up for this loss of pressure metal.

In the case where the casting metal in the mold cavity 87, illustrated in Figure 13, is a metal having a specific gravity less than the specific gravity of the pressure metal, then before the pressure metal is introduced upon the surface of the casting metal, a thin metal disc may be inserted in the mold filling opening 91 that closely fits the wall thereof and rests upon the surface of the casting metal. In this instance, the metal disc will bend and conform to the shape of the recess 101 as the casting metal shrinks during the cooling process so that hydraulic pressure can be continuously maintained upon the casting metal during the cooling process in the same manner as heretofore described with regard to the functioning of the metal discs 80 and 81, illustrated in Figures 9 to 12, inclusive.

In all of the illustrations thus far described it will be noted that the mold filling opening is relatively large so that the quantity of casting metal retained in this mold filling opening is 75 relatively large and therefore will retain a large

quantity of heat during the cooling operation, particularly so since the cooling passages in the mold members have been arranged so that they will not extract a large quantity of heat from the area of the mold filling opening until after the main body of the casting has solidified whereby the casting metal in the mold filling opening will be maintained in a fluid condition until the last part of the cooling cycle. It is, of course, within the purview of this invention that a plurality of cooling passages could be provided around the mold cavity and cooling fluid be passed therethrough sequentially or progressively as the casting metal cools so that the cooling of the metal in the mold filling opening will be occasioned during the last portion of the cooling cycle.

In working the process of this invention the principal feature is to control the cooling of the casting so that the casting metal in the mold filling opening will be the last to solidify and thereby hydraulic pressure can be constantly maintained on the casting metal because the pressure metal will be at a lower melting temperature than the casting metal and will always be in a fluid condition while it is within the mold filling opening and even though the casting metal has completely solidified. It is, of course, understood that at no time will the temperature in the mold be below the melting temperature of the pressure metal except as illustrated in Figure 13 after the casting metal has completely solidified.

However, the applicant's invention is not confined strictly to a mold having a mold filling opening of a large diameter, but rather the process of this invention is applicable to any mold or die having a small sprue with connecting runners to one or more casting articles if in the practice of this invention the quantity of casting metal that is introduced into the mold is controlled to the extent that the casting metal will completely fill the mold cavity or cavities in which the articles are to be produced but will not fill the sprue and runners. The low temperature pressure metal will be introduced into the sprue and runners so that hydraulic pressure developed within the main cylinder containing the main body of pressure metal will be transmitted constantly through the sprue and runners to the casting metal in the various parts of the mold.

This arrangement has been particularly illustrated in connection with the die casting apparatus shown in Figures 14 and 17, inclusive. In this apparatus there is provided a metal pot 103 that contains a body of molten casting metal 108, the pot being heated by means of an electric heating coil 107. Suitable heat insulating walls 109 are provided around the metal pot 103.

A cylinder 109 extends into the metal pot 103 and has a cylinder bore 110 to receive a plunger 111 that is operated by means of a hydraulic motor in any conventional manner. The upper end of the cylinder 109 has a filling opening in which there is placed a rotary valve 113 that is adapted to close the opening 112 for purposes of operation to be hereinafter described. The cylinder 109 is also provided with a spout 114 that has a rotary valve 115 therein.

The rotary valve 115 is provided with a cut away portion 116 that is adapted to align with the discharge opening 117 in the spout 114 to

permit passage of molten metal from the cylinder 109 into the spout 114.

The cylinder 109 has a cylinder bore 118 that is adapted to receive a body of metal 119 that melts at a lower temperature than the casting metal 108 so that the heating coil 107, which also surrounds the cylinder 109 will retain the pressure metal 119 in a molten condition at all times.

The spout 114 is provided with a nose 120 that engages a socket 121 in a mold member 122 in more or less conventional manner that is now common practice in the die casting machine art. The nozzle 120 has an opening 123 that communicates with a tapered sprue 124 provided in the mold member 122, the taper on the sprue 124 having its apex toward the nozzle opening 123.

A second mold member 125 is associated with the mold member 122 and each has a recess therein, or a plurality of recesses, forming one or more mold cavities 126. The mold members 125 and 122 are provided with cooling passages 127 and 128, respectively, that are arranged around the mold cavity 126 in such a manner that the casting metal that is transferred into the mold cavity 126 is cooled from the outer periphery of the mold cavity toward the sprue 124 so that the casting metal in the sprue will be the last of the casting metal to completely solidify. This is in accordance with the practice previously described in connection with the general description of the process whereby it is possible to constantly maintain hydraulic pressure on the body of casting metal as it cools and thus follows any shrinkage of the metal.

In the operation of the apparatus illustrated in Figures 14 and 15, the valves 116 and 113 are first placed in position as illustrated in Figure 14, the plunger 111 being in full retracted position as shown therein. The casting metal having a lower specific gravity than the pressure metal, may then enter the cylinder bore 118 through the valve 113 and the passage 112 so that the casting metal will float upon the pressure metal 119. Since the valve 115 now has the solid portion 129 thereof across the passage 114, the cylinder bore 118 will receive a predetermined quantity of casting metal. The exact quantity of casting metal filled into the cylinder bore at each filling operation can be readily controlled either by means of the liquid level of the pressure metal 119 or by means of the position of the plunger 111 to increase or decrease the volume of the space above the level of the pressure metal 119.

When the upper portion of the cylinder bore 118 has completely filled with casting metal, the valve 113 will be closed and the valve 116 will be opened, as illustrated in Figure 15. The plunger 111 will then be advanced into the cylinder bore 118 thereby causing the pressure metal 119 to raise the casting metal through the passage 114 and through the sprue 124 into the mold cavity 126. The casting metal will completely fill the mold cavity 126 and may partially enter the sprue 124 to a level indicated by the liquid line 130. The low temperature pressure metal will fill the remaining portion of the sprue 124 and will extend back into the cylinder bore 118 through the passage 114.

Since the cooling of the casting in the mold cavity 126 proceeds from the outer periphery of the casting toward the sprue 124 it will be apparent that portion of the casting metal adjacent the sprue 124 will be the last of the casting metal to solidify so that with the pressure metal 119 constantly applying pressure upon the casting

metal that the pressure will be transmitted to the casting metal as it is solidifying and thus increase the density of the casting metal and prevent any porosity due to shrinkage of the casting metal. As soon as sufficient time has elapsed to permit complete solidification of the casting metal, including that small portion in the sprue, the plunger 111 will be retracted to permit the pressure metal to drop back into the cylinder bore 118. The mold may then be opened and the casting removed.

By the process of this invention it is, therefore, possible to secure more dense casting articles by the die casting method using the process of this invention than according to the conventional practice wherein the same casting metal is used in an effort to hold pressure through the goose-neck, the sprue and into the mold cavity. The use of metals having a different melting temperature, wherein the pressure metal has the lower melting temperature permits complete solidification of the casting metal without critically controlling the temperature reduction of the casting metal, as would be required if a single metal was used in the process and the general cooling arrangement disclosed herein was attempted. It would be exceedingly difficult to have the same metal in the nozzle passage 123 and in the sprue 124 and so accurately control the cooling of the casting in the mold cavity 126 that only that metal in the casting and down to the liquid level 130 would solidify and the remainder of the metal in the sprue 124 would remain in a liquid condition. With a substantial temperature differential between the casting metal and the pressure metal, the cooling of the casting metal can be controlled in a manner heretofore described to complete solidification without any solidification of the pressure metal, so that the hydraulic pressure produced by the pressure metal will be retained on the casting metal throughout the cooling process.

As a further illustration of the use of this process of casting metal under pressure for producing a plurality of individual casting, the mold illustrated in Figure 17 is constructed with a plurality of individual casting cavities 131 that are connected to a sprue 132 by means of runners 133. In this instance cooling passages 134 may be provided only in the upper die member 135, the lower die member 136 containing the sprue and runners 132 and 133. In practicing the process of this invention to produce individually cast articles as illustrated in Figure 17, the quantity of casting metal is predetermined in accordance with the practice heretofore described so that the quantity of casting metal that is carried into the molds by the pressure metal is sufficient to fill the individual casting cavities 131, but there will be only a slight excess. In fact, the pressure metal will fill the sprue 132 and substantially fill the runners 133 to the liquid level 131.

Since the cooling passages 134 are only in the upper mold member 135 it will be quite apparent that the castings 131 will cool from the top side down and that therefore the casting metal in the lower portion of the mold cavities 131 will be the last to solidify so that the liquid pressure metal in the runners 133 will constantly maintain hydraulic pressure upon the casting metal as it solidifies and therefore increase the density of the same and follow the shrinkage of the metal to maintain constant density throughout the entire casting.

The bottom wall 138 of the runners 133 is tapered downwardly toward the sprue 132 so that when the plunger 111 is retracted the pressure

metal in the runners and the sprue 133 and 132 will drop into the cylinder bore 118.

As a further exemplification of the process of this invention, Figure 18 illustrates an apparatus wherein the process is used for extrusion molding continuous length strips. The apparatus herein consists of a cylinder 140 having a cylinder bore 141 that receives a plunger 142 extending from a double-acting hydraulic motor 143 for reciprocating the same within the cylinder bore 141. The hydraulic motor 143 is secured to the cylinder 140 by means of strain rods or bolts 144.

A suitable pressure actuated system is provided for the double-acting hydraulic motor 143 and may consist of a pump 145 that may be of any conventional type such as a constant pressure variable delivery pump of any of the well-known constructions. The pump 145 is, of course, driven by a suitable power source. The pump 145 receives pressure fluid from a reservoir 146 through a conduit 147 and delivers the same under pressure to a conduit 148 that supplies a 4-way valve 149 that is regulated by means of a control handle 150 for delivering fluid under pressure to the supply lines 151 and 152 that are connected to opposite ends of the hydraulic motor 143 for supplying fluid under pressure thereto in the well-known and conventional manner to produce reciprocation of the plunger 142. The 4-way valve 149 is provided with a return conduit 153 that is connected to the reservoir 146 for returning pressure fluid to the reservoir from either of the conduits 151 and 152 according to the setting of the 4-way valve, this circuit being a conventional hydraulic control circuit.

The cylinder 140 is provided with an inlet chamber 154 that is connected to a supply reservoir 155 by means of a connecting conduit 156. A swinging check valve 157 is provided in the inlet chamber 154 to close the conduit 156 when pressure is created in the chamber 154, the check valve 157 opening only in a rightward or counter-clockwise direction. A discharge chamber 158 is provided on the cylinder 140 and is disposed on the opposite side thereof from the inlet chamber 154, the discharge chamber 158 being connected to a die or forming chamber 159 in any suitable manner. A heat insulating material 160 is disposed between the discharge chamber 158 and the die or forming chamber 159. The cylinder 140, the inlet chamber 154 and the discharge chamber 158 are heated by means of an electric coil 161 that is adapted to maintain the body of metal within the chambers in a molten condition at all times. These chambers are enclosed by a suitable heat insulating material 162.

The reservoir 155 that contains a quantity of metal in molten condition is heated by means of an electric heating coil 163 and has heat insulating material 164 surrounding the same to prevent heat loss therefrom.

The reservoir 155 is provided with a cover 165 secured thereto in any suitable manner and has a filling opening 166 through which molten metal can be passed into the chamber or reservoir 155, the opening 166 being closed by a cover member 167. A conduit 168 extends through the cover member 165 for conducting an inert gas into the chamber to prevent oxidation of the molten metal in the chamber, a check valve 169 providing means for the escape of air or a small quantity of inert gas if it is desired to circulate the same through the reservoir chamber 155. A valve member 170 is carried upon the end of a rod 171 that extends through the top cover

165 and terminates in a ring 172 to permit lifting of the valve 170 from its seat 173 provided on the inlet end of the conduit 156, whereby the conduit 156 can be closed from the body of molten metal in the reservoir 155 when desired. A lever 174 is pivoted to the ring 172 by means of a pin 175 that can be swung into engagement with the top cover 165 to hold the valve 170 in an upward position as illustrated in Figure 18. A vent valve 176 is provided in the top of the cylinder 140 to vent air that may be entrapped therein when the machine is first started or to permit venting of gases that may accumulate in the top of the cylinder during the operation of the machine. The vent valve 176 is closed by means of a spring 177 that retains the same closed at all times except when pressure is applied upon the top side of the valve to force the same downwardly for venting purposes.

The extrusion die or forming chamber 159 is provided with cooling passages 178 extending throughout the length thereof having fluid supply connections 179. The extrusion die or forming chamber 159 may be of any suitable length for cooling and solidifying the molten metal as it passes through the chamber 159. The extrusion opening 180 may be of any desired cross section to produce the desired article in any well-known fashion.

In the operation of the machine in Figure 18 a body of molten metal 181 is placed in the lower end of the cylinder 140 and is maintained in a molten condition at all times by means of the heating coil 181. This body of molten metal has a lower melting temperature than the metal that is to be extruded and also has a greater density than the metal to be extruded so that it will always remain in the bottom of the cylinder 140. As an example, this pressure metal 181 may be lead having a melting temperature of 621° F. and a specific gravity of 11.34. The metal to be extruded is initially placed in the reservoir 155 and brought to a molten condition therein. Subsequently, the valve 170 will be opened to permit the molten metal to flow through the conduit 156, the check valve 157 and into the chambers 154, 158 and the cylinder bore 141, whereby the metal to be extruded will float upon the surface of the pressure metal 181. The metal to be extruded is one that has a higher melting temperature than the pressure metal and has a low specific gravity so that it will always float upon the pressure metal. As an example, the metal to be extruded may be aluminum having a melting temperature of 1217° F. with a specific gravity of 2.7 or may be one of the cast or gray irons having a melting temperature of 1900° F. to 2200° F. with specific gravities of 7.03 to 7.13.

As soon as the molten metal to be extruded enters and fills the cylinder bore 141 and the discharge chamber 158, the hydraulic motor 143 will be operated to advance the plunger 142 into the cylinder bore 141 thereby producing hydraulic pressure upon the extruding metal by means of the pressure metal 181. The check valve 157 closes so that the molten extrusion metal is forced outwardly through the extrusion opening 180. In its passage through the extrusion chamber 159 and the extrusion opening 180, the metal is gradually cooled from its molten condition through successive stages of a slush, semisolidity and a solid material so that when it passes from the extrusion opening 180 the metal will be in a substantially solid condition. The plunger 142 is permitted to stroke upwardly until the surface level

182 of the pressure metal 181 approaches the bottom level of the inlet and discharge chambers 154 and 158. The hydraulic motor 143 is then reversed to drop the plunger 142 and permit the pressure metal to fall back into the cylinder bore 141, whereupon molten extrusion metal from the reservoir 155 will pass through the conduit 156 and open the check valve 157 to pass into the chamber 154 and again fill the chamber 154 and the cylinder bore 141 with a fresh charge of molten extrusion metal. The hydraulic motor 143 can then make another stroke of operation.

Due to the fact that the body of metal in the extrusion chamber 159 is gradually passing through a stage from a molten metal to a solid metal throughout a substantial length of the chamber 159, the intermittent operation of the machine, while stopping the actual extrusion of the solid metal from the end of the extrusion opening 180, will have no detrimental effect on the continuous extrusion of the metal because each charge can knit thoroughly with a previous charge because of the gradual change that occurs in the condition of the metal through the extrusion chamber, it being remembered that molten metal in each instance is being supplied into the extrusion chamber to knit with molten metal that is already there.

By the use of the process heretofore described, the pressure metal 181 may maintain hydraulic pressure on the metal that is being extruded as long as there is any movement of the metal in the extrusion chamber so that the density of the metal in the extruded member will be substantially constant. It will also be apparent that since the metal is gradually cooling as it passes through the extrusion chamber, and the metal most remote from the filling opening from the discharge chamber is that which is solidified, that hydraulic pressure will be continuously maintained on that body of the metal that is in the process of solidification so that during the solidification of the metal, pressure is retained thereon to increase the density of the metal and absorb any shrinkage that occurs due to the solidification. This, of course, is in accordance with the general process heretofore described wherein hydraulic pressure is continually maintained on the body of casting metal while it is in process of cooling and solidification.

In describing the process there has been incorporated herein several examples of metals that can be used in practicing the process, but it is to be understood that the process is not limited to the specific examples set forth but that other metals and other alloy of metals can be used in the practice of the process. Also, while in the general description of the process it has been stated that the metals are to be of different specific gravity, yet it is entirely within the purview of this invention that the metals may be of practically the same specific gravity and with their temperatures substantially divergent, for if the metals are of substantially the same specific gravity they may be separated by a quiescent working of the molten metals to prevent substantially any agitation therebetween whereby to keep them separated or the disc means may be used to prevent their intermixing. The temperature differentials between the metals should be sufficient to permit the functioning of the process without critical control.

While the process disclosed and described herein and the apparatus constitutes the preferred forms of the invention, yet, it is to be

understood that the process as well as the apparatus can be varied without going beyond the general scope of the spirit of the invention, and that all such modifications of the invention that fall within the scope of the appended claims are intended to be included herein.

Having thus fully described my invention what I claim as new and desire to secure by Letters Patent is:

1. A process of pressure casting molten metal that includes, introducing a molten metal into a mold until the casting cavity in the mold is full and the molten metal stands partially in the filling opening for the mold, introducing a second molten metal having a lower melting temperature than the first metal into the unfilled portion of the filling opening of the mold, and applying pressure upon the second metal to condense the first metal thereby and retain pressure thereon throughout the entire cooling period of the first metal.

2. The process of molding metal under pressure that includes, filling a mold cavity with a molten metal until the level of the molten metal reaches into the filling opening of the mold cavity, introducing a second molten metal under pressure maintained at a lower melting temperature than the first metal into the mold filling opening for applying pressure upon the first metal, cooling the first metal from the outer periphery of the mold cavity toward the filling opening thereof whereby the most liquid metal will always be toward the filling opening, and maintaining pressure upon the first metal by means of the second metal until the first metal has completely solidified.

3. The process of pressure casting molten metal in a mold cavity that includes, filling a mold cavity with sufficient molten metal whereby to produce a complete casting but wherein the molten metal will not completely fill the mold cavity filling opening, introducing a second molten metal under pressure into the mold to completely fill the mold filling opening whereby to apply hydraulic pressure upon the first molten metal in the mold cavity, said second molten metal having a lower melting temperature than the first molten metal whereby it retains its molten condition at all times during the casting process, and withdrawing heat from the molten metal within the mold cavity in such a manner that the solidification of the metal within the cavity proceeds toward the mold filling opening whereby hydraulic pressure is constantly maintained on the metal in the cavity when solidifying within the mold.

4. The process of pressure casting metal that consists of, retaining a body of metal in molten condition within a cylinder, introducing a casting metal having a higher melting temperature than the first metal upon the body of the first metal and which is supported thereby, applying pressure upon a relatively large portion of the first body of molten metal to produce movement thereof and transfer the casting metal into a mold together with a small portion of the first metal that enters the filling opening of the mold, maintaining pressure upon the first metal whereby to produce hydraulic pressure thereby that is constantly maintained on the body of the molten metal in the mold as solidifying and until completely solidified.

5. The process of pressure casting metal that includes, maintaining a body of molten metal within a chamber, placing a second body of molten metal having a higher melting tempera-

ture and a lower specific gravity than the first molten metal within the chamber and upon the first metal to be supported thereby, applying pressure upon a relatively large portion of the first metal to transfer the second metal from the chamber into a mold cavity together with a small portion of the first metal that remains in the filling opening for the mold cavity, abstracting heat from the second metal within the cavity in such a manner as to solidify the second metal from the outer extremities of the mold cavity toward the filling opening, and maintaining pressure on the first metal during the solidification of the second metal whereby to maintain hydraulic pressure upon the second metal in the mold cavity as it solidifies.

6. The process of die casting which consists of, providing a body of molten metal within a chamber within which pressure is adapted to be produced, introducing a second body of molten metal into the chamber having a higher melting temperature than the first metal for flotation upon the first metal, applying pressure upon a relatively large portion of the first metal to transfer the second metal from the chamber into a mold together with a quantity of the first metal that remains in the sprue of the mold, and withdrawing heat from the metal within the mold in such a manner that solidification progresses toward the sprue whereby pressure maintained upon the first metal will be constantly transmitted to the metal in the mold as it solidifies.

7. The process of simultaneously pressure casting a plurality of cast articles from molten metal that includes, providing a body of molten metal within a chamber, introducing a predetermined quantity of casting metal into the chamber for flotation upon the first metal and having a higher melting temperature than the first metal, said predetermined quantity of casting metal being sufficient to fill the mold cavities to produce the plurality of articles and only a slight excess, and applying pressure upon the first metal to transfer the casting metal into the individual mold cavities for simultaneously producing a plurality of cast articles, said first metal entering the sprue and runners of the mold whereby to maintain pressure on the cast articles constantly while the casting metal is solidifying.

8. An apparatus for die casting that includes, a metal pot for holding a supply of molten die casting metal, means forming a chamber having a portion thereof disposed within the metal pot, an inlet passage in said chamber forming means through which molten metal from said pot can pass into said chamber, valve means for opening and closing said passage means, a discharge spout extending from said chamber, valve means in said discharge spout for opening and closing the same, a body of molten metal within the lower portion of said chamber having a lower melting temperature than said casting metal which is floated thereupon upon opening of said inlet valve, and plunger means reciprocable in said chamber for applying pressure upon said low temperature metal to transfer casting metal from said chamber through said spout into a mold adapted to be associated therewith and carry said low temperature metal into said spout to fill the same when casting said casting metal within a mold cavity.

9. An apparatus for die casting that includes, a metal pot for holding a supply of molten die casting metal, means forming a chamber having a portion thereof disposed within the metal pot,

an inlet passage in said chamber forming means through which molten metal from said pot can pass into said chamber, valve means for opening and closing said passage means, a discharge spout extending from said chamber, valve means in said discharge spout for opening and closing the same, a body of molten metal within the lower portion of said chamber having a lower melting temperature than said casting metal which is floated thereupon upon opening of said inlet valve, a mold positioned in operative association with said spout having a mold cavity therein provided with a sprue to receive molten metal from said spout, plunger means reciprocable in said chamber to apply pressure upon said low temperature metal and transfer said casting metal into said mold cavity and dispose said low temperature metal in said spout and in a portion of said sprue to thereby maintain pressure on the metal in said cavity, and means for withdrawing heat from said mold in such a manner that the casting metal therein solidifies from the outer extremities of the mold cavities toward the sprue.

10. An apparatus for die casting that includes, a metal pot for holding a supply of molten die casting metal, means forming a chamber having a portion thereof disposed within the metal pot, an inlet passage in said chamber forming means through which molten metal from said pot can pass into said chamber, valve means for opening and closing said passage means, a discharge spout extending from said chamber, valve means in said discharge spout for opening and closing the same, a body of molten metal within the lower portion of said chamber having a lower melting temperature than said casting metal which is floated thereupon upon opening of said inlet valve, a mold positioned in operative association with said spout having a plurality of individual mold cavities therein provided with runners connected with a sprue to receive molten metal from said spout, plunger means reciprocable in said chamber to apply pressure upon said low tem-

perature metal and transfer said casting metal into said mold cavities and dispose said low temperature metal in said spout and in said sprue and a portion of said runners to thereby maintain pressure on the metal in said cavities, and means for withdrawing heat from said mold in such a manner that the casting metal therein solidifies from the outer extremities of the mold cavities toward the sprue.

10. The process of simultaneously pressure casting a plurality of cast articles from molten metal that includes, introducing a predetermined quantity of casting metal into a mold to fill the several cavities therein with only a slight excess, introducing a second molten metal having a lower melting temperature into the sprue and runners of the mold through which the first metal was introduced, applying pressure upon the second metal to produce hydraulic pressure upon the 20 first metal, withdrawing heat from the first metal in such a manner that it solidifies toward the level between the metals whereby the second metal continuously maintains hydraulic pressure on the first metal while it is solidifying.

MORRIS F. BOOTH.

#### REFERENCES CITED

The following references are of record in the file of this patent:

| UNITED STATES PATENTS |          |               |
|-----------------------|----------|---------------|
| Number                | Name     | Date          |
| 755,722               | Stroh    | Mar. 29, 1904 |
| 1,219,358             | Stewart  | Mar. 13, 1917 |
| 35 1,486,751          | Hult     | Mar. 11, 1924 |
| 1,912,981             | Hoy      | June 6, 1933  |
| 1,971,652             | Haessler | Aug. 28, 1934 |
| 2,143,323             | Korsmo   | Jan. 10, 1939 |
| 40 2,339,265          | Held     | Jan. 18, 1944 |

#### FOREIGN PATENTS

| Number  | Country       | Date         |
|---------|---------------|--------------|
| 204,743 | Great Britain | Oct. 8, 1923 |